

Jan. 1, 1957

F. J. ZIMMERMANN

2,776,069

CONTAINER FOR LIQUEFIED GAS

Filed June 30, 1955



HEAT TRANSFER VS. CALORIMETER PRESSURE

FIG. 2



FIG. 1

INVENTOR.  
FRANCIS J. ZIMMERMANN  
BY *Douglas M. Kryder*  
AGENT

1

2,776,069

**CONTAINER FOR LIQUEFIED GAS**

Francis J. Zimmermann, West Roxbury, Mass., assignor to Arthur D. Little, Inc., Cambridge, Mass., a corporation of Massachusetts

Application June 30, 1955, Serial No. 519,075

6 Claims. (Cl. 220—9)

This invention relates to dewar-type containers and more particularly to improved surfaces for the lining of the vacuum chamber of the dewar-type containers.

In recent years many industrial processes and research projects have come to be carried out at temperatures at least as low as that attained by the use of liquid nitrogen (below  $-195.8^{\circ}$  C. or  $77.3^{\circ}$  K.). The handling, storing and transporting of the low temperature liquids required in such processes and research must be done by means of large (usually 25-liter capacity) dewar-type flasks which contain an inside vessel which has a complete double wall with the area between being evacuated. This vacuum chamber is the primary means of insulating the inside vessel and the liquefied gas or gases which it contains from the outside ambient temperature. The emissivity and heat transfer properties of the surfaces of these walls which face inward into the evacuated area of this vacuum chamber are of primary importance in designing an efficient dewar-type flask. This is due to the fact that often the major source of heat leakage in such a container is due to radiation heat transfer.

Although the description of this invention will be given hereinafter in terms of a dewar-type container or flask suitable for handling liquefied gases or liquids at temperatures of the order of liquid nitrogen or even liquid helium, the principle of depositing a finish showing extremely low emissivity and heat transfer is equally applicable to construction of other vessels, tank cars and apparatus used for handling extremely cold liquids by insulating them by a surrounding evacuated area.

Heretofore it has been customary to coat the facing inside walls of the vacuum chamber or jacket with a silver solution, if glass apparatus were used, to reduce emissivity and radiant heat transfer. Although this did materially cut down the loss of liquid gases due to vaporization in glass dewars, it was desirable to find an efficient means of treating these inside walls in the case of metal dewars. By the process of this invention it is possible now to reduce heat transfer across the vacuum jacket to not more than one-half that shown by previous methods of surface treatment.

It is therefore an object of this invention to provide the inside walls of a vacuum jacket or those enclosing an evacuated area with surfaces which have emissivities markedly lower than heretofore achieved. It is another

2

object to provide such walls with surfaces which show markedly lower radiant heat transfer than previously achieved. It is a further object of this invention to provide more efficient dewar-type flasks, storage vessels and transfer lines for handling liquefied gases, or liquids which must be kept at very low temperatures.

The means for achieving this invention will be shown by the following discussion and with reference to the accompanying drawings in which

10 Fig. 1 is a cross-section of a typical dewar-type flask or container embodying this invention; and

Fig. 2 is a plot of heat transfer as related to calorimeter pressure for two surface treatments.

Surfaces of extremely low emissivity are achieved in the process of this invention by electroplating the surface by means of a silver plating process. The surfaces are given a very brilliant luster and are not further treated by buffing or other form of rubbing or polishing.

Fig. 1 shows a cross-section of a typical dewar-type container for liquefied gases such as air, nitrogen, oxygen, or hydrogen. The vacuum jacketed vessel with outer wall 12 and inner wall 16 and containing the liquefied gas 14, is suspended inside a metal container 10 and held in place by a neck ring 17. The inside area 13 between walls 15 and 16 of the vessel 15 is evacuated, and the inside surfaces 11 and 12 are treated to reduce their emissivity. The improvements in efficiency in a dewar-type container are achieved by the process of this invention by treating these surfaces 11 and 12.

20 The treatment of surfaces 11 and 12 consists of depositing a silver finish by electroplating from a bright plating bath to give an essentially mirror-bright coating, i. e., a coating having a reflectivity substantially the same as that of a mirror. A potassium cyanide plating bath

25 containing organic addition agents such as for example thiourea, to contribute a positive brightening effect and to reduce grain size has been found satisfactory for depositing the necessary brilliant silver coating. Variables such as composition, current density and agitation may be

30 determined experimentally to give the maximum brilliance to the final surface.

It is essential that no buffing step be used in obtaining the brilliant surface of this invention. Extensive tests have shown that when electroplated surfaces are buffed 45 their emissivities and their ability to transfer radiant heat are markedly increased, thus decreasing their efficiencies for such uses as considered here. Although the reason for this is not precisely known, it is known that buffing does change a surface's physical properties such as its electrical resistance.

The inner and outer shells may be of any suitable metal such as stainless steel or copper or of a rigid plastic material coated with a conducting film suitable to serve 50 as an electrode in the plating bath.

Although the thickness of the silver finish formed on these surfaces does not appear to be critical, it is desirable to maintain it at a minimum from an economic point of view. Thicknesses of approximately 0.0003 inch have been found to be very satisfactory.

The vacuum jacket of a 25-liter liquid nitrogen dewar, such as is illustrated in Fig. 1, was used as a modified calorimeter to measure the relative effectiveness of various surfaces. The calorimeter was so set up and instrumented that the amount of vacuum within the evacuated area, corresponding to area 13 in Fig. 1, could be varied, the quantity of liquid boiled off could be measured and the amount of radiant heat transferred from surface 12 to surface 11 could be measured.

Heretofore, gold-plated finishes had been considered effective and efficient surfaces for metal vacuum-jacketed vessels in dewar-type containers. In Fig. 2 there are plotted data showing the variation of heat transfer with pressure in the evacuated area. The heat transferred at zero pressure is essentially due to radiation in this apparatus. It will be seen from Fig. 2 that in this test the bright silver finish of this invention transfers by radiation just about one-half the amount of radiant heat transferred by the gold plated surfaces when the data lines are extrapolated to zero mm. Hg.

Further testing with the calorimeter was carried out by coating the surfaces involved in various ways and measuring the emissivity factors. These factors were obtained by measuring the amount of boil-off liquid nitrogen when the outside of the vacuum jacket was at room temperature. From these data the amount of heat transferred across the vacuum jacket (and hence by the treated surfaces) could be calculated; and from this the emissivity factor which is in a direct ratio to the heat transferred by radiation in the equipment to the heat that would be transferred if both surfaces were black-bodies could be determined.

The resulting data are shown in the table in which there is indicated the relative merit of various combinations of surfaces. All of the surfaces except the polished copper and stainless steel were electroplated. Most of the tests combined a polished gold-plated shell with spheres of various treatments in order that an indication of the relative emissivities of the nitrogen cooled surface (represented by surface 11 of Fig. 1) would be shown directly by the emissivity factor.

It is readily seen that two silver surfaces prepared in accordance with this invention are the best combination, having a heat leakage approximately one-half that of two polished gold surfaces. However, if only the surface facing the evacuated area of the wall which comes in contact with the liquid to be stored or handled is coated to give a finish as described by this invention, the emissivity factor is reduced to 0.0061 (weighted average) if the surface of the outer wall is finished in polished gold. This should be compared with 0.0103 (weighted average) for both surfaces being finished in polished gold.

It will be seen from the examples and data shown in Table I that the brilliant unbuffed silver finish for both the inside surfaces of the vacuum jacket shows a marked increase in efficiency over any of the finishes used heretofore, including polished gold. Such increased efficiency is shown by the fact that heat transfer, and also emissivity, is reduced by the brilliant silver surfaces of this invention to about one-half that shown by the best previous surfaces. Thus, by using the surface finishes of this invention it is possible to make dewar-type containers which can store or transport liquefied gases with far less loss of the liquid by boil-off. Such savings resulting from the dewar-type containers of this invention can be realized in the form of smaller losses or ability to store the liquefied gases over a longer period. Although the characteristics of this invention have been described in terms of dewar-type containers, the principle of applying brilliant, unbuffed silver finishes to attain low emissivity and low heat transfer may be applied to large vacuum-jacketed storage vessels, trailer trucks and other jacketed apparatus, such as transfer lines, which are required to insulate liquefied gases or other liquids which must be handled at very low temperatures.

TABLE I  
*Emissivity factors for various combinations of the inner surfaces of an evacuated vessel*

| 5  | Sphere Surface<br>(Liquid N <sub>2</sub> Temperature) <sup>b</sup> | Shell Surface (Room Temperature) <sup>a</sup> |                               |                 |                    |
|----|--------------------------------------------------------------------|-----------------------------------------------|-------------------------------|-----------------|--------------------|
|    |                                                                    | Brilliant<br>Unbuffed<br>Silver               | Polished<br>Gold              | Matte<br>Silver | Polished<br>Copper |
| 10 | Brilliant unbuffed silver-----                                     | .0054                                         | { .0061<br>d. 0063<br>d. 0060 | .0059           | -----              |
| 15 | Matte silver -----                                                 | -----                                         | .0030                         | -----           | -----              |
| 15 | Dry buffed silver-----                                             | -----                                         | .0093                         | -----           | -----              |
| 15 | Matte gold -----                                                   | -----                                         | .0033                         | .0083           | -----              |
| 15 | Gold wash-----                                                     | -----                                         | .0092                         | -----           | -----              |
| 15 | Dry buffed gold-----                                               | -----                                         | .0096                         | -----           | -----              |
| 20 | Polished gold-----                                                 | -----                                         | { .0100<br>d. 0110            | -----           | -----              |
| 20 | Polished copper-----                                               | -----                                         | .0092                         | -----           | .0087              |
| 20 | Stainless steel spinning—<br>rubbed with fine emery<br>cloth-----  | -----                                         | d. 0180                       | -----           | -----              |
| 20 | Drafting tape-----                                                 | .0170                                         | .0225                         | -----           | -----              |

<sup>a</sup> Corresponds to surface 12 of Fig. 1.

<sup>b</sup> Corresponds to surface 11 of Fig. 1.

25 The term "matte" is used to describe a finish which is somewhat cloudy or "milky" in appearance.

d Stainless steel sphere—all other copper sphere.

I claim:

1. Walls enclosing an evacuated area, the surfaces of said walls facing each other having a brilliant unbuffed silver finish; said silver finish having been deposited by electroplating from a potassium cyanide bath containing organic additives which reduce the particle size of the silver in said silver finish and which contribute a positive brightening effect.
2. A dewar-type container equipped with a vacuum-jacketed inner vessel for handling liquefied gases, the walls of said vessel facing the evacuated area having a brilliant unbuffed silver finish, said silver finish having been deposited by electroplating from a potassium cyanide bath containing organic additives which reduce the particle size of the silver in said silver finish and which contribute a positive brightening effect.
3. A dewar-type container in accordance with claim 2 wherein said walls are stainless steel.
4. A dewar-type container in accordance with claim 2 wherein said walls are copper.
5. A dewar-type container in accordance with claim 2 wherein said walls are a rigid plastic material covered with a conducting coating.
6. A dewar-type container equipped with a vacuum-jacketed inner vessel for handling liquefied gases, the wall of said inner vessel which is in contact with said liquefied gases having its surface facing the evacuated area coated with a brilliant unbuffed silver finish, said finish having been deposited by electroplating from a potassium cyanide bath containing organic additives which reduce the particle size of the silver in said silver finish and which contribute a positive brightening effect.

60 References Cited in the file of this patent

UNITED STATES PATENTS

- 1,816,476 Fink et al. ----- July 28, 1931  
2,396,459 Dana et al. ----- Mar. 12, 1946  
65 2,643,021 Freedman ----- June 23, 1953

FOREIGN PATENTS

- 483,207 Great Britain ----- Apr. 13, 1938

70 OTHER REFERENCES

Egberg et al.: Article "Brighteners in Silver Plating Solutions," printed by The Electrochemical Society, preprint 74-13, released October 17, 1938, pages 195, 197-75 199.